

## UNITED STATES PATENT OFFICE

2,466,672

COATING COMPOSITION CONTAINING A  
FATTY ACID ESTER AS A GEL STABILIZ-  
ING AGENTEmile E. Habib, Belmont, and David G. Greenlie,  
Wayland, Mass., assignors to Dewey and Almy  
Chemical Company, North Cambridge, Mass., a  
corporation of MassachusettsNo Drawing. Application May 20, 1947, Serial No.  
749,340. In Canada May 11, 1944

7 Claims. (Cl. 260—23.5)

1

This invention relates to coating compositions particularly to compositions of wax and other materials designed to be spread on cardboard, paper or fabrics to make the material moisture and vaporproof.

Paraffin wax has commonly been used for this purpose but paraffin wax does not make a completely moistureproof coating because water vapor may pass through the coating along the paraffin crystal boundaries. To prevent moisture from penetrating, a carton waterproofing material which impregnates cardboard is not as satisfactory as one which forms a continuous film on the surface of the carton provided the surface film is flexible. The reason is that when all of the free space in the cardboard is occupied by wax and the carton is then dented or bent, the crystal structure snaps at the point of greatest strain. Although all of the fibres may not be ruptured across the break, passageways are opened which permit moisture to enter. A film, on the other hand, may distort without rupture. The carton does not split or tear as easily because the fibres are free to move in the free space between the fibres and are not immediately sheared by an impact as happens when fibres are rigidly held in a matrix of impregnating material.

A composition which coats rather than impregnates the board also has advantages because of its economy. Less material is required to coat the board than to impregnate the whole mass. Paraffin, however, impregnates paperboard and consequently certain compositions have appeared in an attempt to modify paraffin so that it will form surface films on the board yet not impregnate it to any substantial degree. Among the more satisfactory compositions for this purpose are mixtures of paraffin or petroleum waxes and an especially depolymerized rubber. Seemingly this combination works because the rubber has gone into a solvated state in the wax and exists in the mixture as a solvated colloidal gel. The gel structure traps and holds the wax on the surface where it solidifies into a continuous film. This coating makes a package which is spectacularly vaporproof, does not block, and is sufficiently flexible to withstand rough handling at room temperatures but the gel when subjected to long continued heating as is necessary when dipping or coating cartons in progress, is unstable.

The objects of this invention are to produce coating compositions which are moisture and vaporproof, which coat rather than impregnate fibrous surfaces, which have high stability in the

2

dipping kettles, which will not sediment, which at the present time require no critical materials in their manufacture and which provide a range of coating compositions from compositions which will neither check nor chip off the board at  $-20^{\circ}$  F. to hard non-blocking coatings at  $+130^{\circ}$  F. Formulas compounded according to the present invention successfully meet these requirements.

Surprisingly, when numerous resins were added to the paraffin in order to increase its viscosity and prevent penetration into the paperboard the rise in viscosity did not inhibit penetration of the compound into the board. In many cases the absorption is even greater when resin is added to the paraffin than when no resin is present. This is characteristic of a wide variety of resins including the coumarone-indene type, rosin, and "Vinsol" resin, the latter being a gasoline insoluble resin derived from the dark colored residue concurrently removed with F. F. wood rosin after extraction of pine chips with a coal tar hydrocarbon such, for instance, as benzene, toluene, xylene (see Patents Nos. 2,287,351 and 2,287,352). It contrasts markedly with the performance of depolymerized rubber. Consequently it was believed that to prevent the penetration of the paraffin into the paperboard a material other than rubber should be one which would peptize and gel in the wax but would not dissolve in it.

If a water insoluble metallic soap be added to paraffin a very marked increase in viscosity is obtained. Of the various stearates, oleates, palmitates, etc., of aluminum, calcium and magnesium, aluminum stearate was found to be the most satisfactory for increasing the viscosity of the material when only a small amount was used. For example, a gel composed of 5% aluminum stearate in paraffin penetrates newsprint scarcely at all. However, if this mixture is maintained at  $200^{\circ}$  F. for forty-eight hours, the original viscosity drops progressively until it is only slightly greater than that of the paraffin. The gel also gradually disappears and the aluminum stearate separates as a flaky sediment. After such ageing, this compound penetrates the board as readily as does uncompounded paraffin wax.

We have discovered that the separation of water insoluble metallic soaps, particularly aluminum stearate, from the compound may be prevented and that a substantially stable viscosity may be given to the compound by adding to the composition fatty-acid esters of mono- and di-anhydro-hexahydric alcohols in which the fatty acid contains from 12 to 18 carbon atoms. Tests

made using all esters which are commercially available at present show that the stabilization imparted to the wax stearate composition is a general property of fatty-acid esters of mono- and di-anhydro-hexahydric alcohols.

We prefer, because of present availability, to use mannide dioleate or its stereoisomer sorbide dioleate, but the following range of materials have already given operative results: mannan mono-oleate, sorbitan mono-oleate, sorbitan dioleate, sorbitan trioleate, sorbitan tetraoleate, sorbitan monostearate, sorbitan distearate, sorbitan tetrastearate, mannide dioleate, mannide monolaurate, mannide dipalmitate, mannide monostearate, sorbide dioleate and sorbitan monolaurate and mixtures of the foregoing.

When these materials are added to the metallic soap-wax composition, excellent stability is achieved. In the first four hours after the addition the viscosity drops slightly. Thereafter the compound may be subjected to holding temperatures of 200° F. in the dip tanks with no precipitation of the gel. For most uses, the paraffin-stearate compound will be found too brittle, but it may be plasticized by the addition of an organic plasticizer. This may be a compatible resin, among others, those listed above, or an appropriate proportion of microcrystalline wax—or both. Because of its availability and constant performance, we prefer polymerized B-pinene.

The term "petroleum wax" is intended to cover the group of wax-like petroleum hydrocarbons including the crystalline paraffin waxes and the so-called "amorphous" or microcrystalline petroleum waxes which frequently are produced by further refining of petrolatum.

The stability which is given to the gel of a metallic soap in petroleum wax by the higher fatty-acid esters described above is imparted to the whole range of such waxes. Our invention contemplates that the wax may either be paraffin or microcrystalline ("amorphous") waxes or mixtures of the two in any proportions which are necessary to give whatever heat or cold resistance may be demanded. The following examples show how the coatings may be adapted to various temperature conditions by a proper selection of the melting point of the waxes and the mutual proportions which are employed. Our preferred examples are given as follows:

#### Example 1

- (a) 57 parts of aluminum stearate, 50 parts of sorbide dioleate are stirred together until the stearate is thoroughly wetted.
- (b) 800 parts paraffin wax (M. P. 135° F.) are heated to 200-210° F.
- (c) Mixture (a) is added to mixture (b) and the temperature is raised to 250-260° F. with stirring. At this temperature the mass gels.
- (d) 80 parts of polymerized B-pinene (M. P. 115° F.) are pulverized and added with stirring to (c).
- (e) 813 parts of paraffin (M. P. 135° F.), 200 parts of amorphous petroleum wax M. P. 158-60° are melted together at 210° F. The product of step (d) is then added to this mixture and stirring is continued until the temperature drops to 175-170° F. The mass is then run out into shipping containers.

This compound will neither check nor chip off paperboard at +5° F. It will not block at +100-115° F. It solidifies at 130-134° F. Its viscosity (cup method) at 175 F. is 13-15 seconds.

#### Example 2

A composition which will not block at +130° F. but resists +20° F. is made by substituting 146° F. M. P. paraffin for the 135° F. M. P. paraffin of Ex. 1.

#### Example 3

A compound which will neither check nor chip off the board at -20 F. but will block at about 110° F. is made by following the same procedure as in Example 1 save for (e) where paraffin wax (M. P. 135° F.), 593 parts, microcrystalline petroleum wax (M. P. 152° F.), 400 parts, are used.

#### Example 4

A compound which remains flexible at -20° F. but blocks at 70° F. is made as follows:

- (a) 1000 parts microcrystalline wax (M. P. 152° F.) are melted at 190-200° F.
- (b) 288 parts aluminum stearate, 242 sorbide dioleate are stirred together until thoroughly wet.
- (c) (b) is added to (a) with stirring and the temperature raised to 250° F. until no lumps appear.
- (d) 370 parts microcrystalline wax (M. P. 152° F.) is heated to 245-250° F. and 100 parts of pulverized polymerized B-pinene added with stirring.
- (e) The product of (d) is added to the product of step (c) and stirred until the temperature drops to 220° F. It is then packaged.

#### Example 5

The stabilizing properties of a series of anhydrohexahydric alcohol fatty acid esters were tested as follows: 100 parts by weight of paraffin wax (M. P. 135° F.) were heated to 170-180° F., and 3.3 parts aluminum stearate stirred into the wax until dissolved. The stabilizing agent was then added and the mixture heated with stirring to 240° F. The viscosity of the mixture was read while hot, again after cooling and remelting, and at successive intervals after storage at elevated temperature. In the storage-stability results, "excellent" denotes a composition which maintained its viscosity throughout the conditions of the test with only slight variations; while "good" refers to a composition whose original viscosity was lowered, but whose final viscosity was substantially higher than that of unstabilized compounds. In no case did the aluminum stearate settle out of the mixture.

| 55 | Stabilizer             | Parts by Weight | Stability on Storage |
|----|------------------------|-----------------|----------------------|
|    | Mannitan mono-oleate   | 1.54            | excellent.           |
|    | Sorbitan mono-oleate   | 1.54            | Do.                  |
|    | Sorbitan dioleate      | 2.66            | Do.                  |
| 60 | Sorbitan trioleate     | 3.89            | Do.                  |
|    | Sorbitan tetraoleate   | 5.30            | good.                |
|    | Sorbitan monostearate  | 1.54            | excellent.           |
|    | Sorbitan distearate    | 2.66            | Do.                  |
|    | Sorbitan tetrastearate | 5.30            | Do.                  |
|    | Mannide dioleate       | 2.93            | good.                |
| 65 | Mannide monolaurate    | 1.32            | Do.                  |
|    | Mannide dipalmitate    | 2.69            | Do.                  |
|    | Mannide monostearate   | 1.67            | Do.                  |
|    | Sorbide dioleate       | 2.93            | excellent.           |
|    | Sorbitan monolaurate   | 1.24            | Do.                  |

Microscopic studies on the crystal structure of the coating show that the size of the crystals is greatly reduced when our invention is practiced. Progressive crystal growth is inhibited, probably because of the presence on the crystal surfaces of a material which is not soluble in the wax. The coatings made from these materials when spread

on cardboard, paper, or fabrics are dense and highly vapor and gas proof.

This application is a continuation-in-part of our co-pending application Serial No. 486,584, filed May 11, 1943, now abandoned.

We claim:

1. A coating composition comprising a petroleum wax, a water-insoluble metal soap, and a gel-stabilizing agent selected from the class consisting of fatty acid esters of mono- and di-anhydro-hexahydric alcohols, the fatty acid containing from 12 to 18 carbon atoms, said composition being in the form of a gel.

2. A coating composition comprising a petroleum wax, a water-insoluble metal soap, a gel-stabilizing agent selected from the class consisting of fatty acid esters of mono- and di-anhydro-hexahydric alcohols, the fatty acid containing from 12 to 18 carbon atoms, and a compatible organic plasticizer, said composition being in the form of a gel.

3. A coating composition comprising a mixture of a paraffin wax, a microcrystalline wax, a water-insoluble metal soap, sorbide dioleate, and a compatible organic plasticizer, said composition being in the form of a gel.

4. A coating composition comprising a petro-

leum wax, aluminum stearate, sorbide dioleate, and polymerized B-pinene, said composition being in the form of a gel.

5. A coating composition comprising a petroleum wax, a water-insoluble metal soap, and an oleic acid ester of an anhydro-hexahydric alcohol, said composition being in the form of a gel.

6. A coating composition comprising a petroleum wax, a water-insoluble metal soap, and a stearic acid ester of an anhydro-hexahydric alcohol, said composition being in the form of a gel.

7. A coating composition comprising a petroleum wax, a water-insoluble metal soap, and a lauric acid ester of an anhydro-hexahydric alcohol, said composition being in the form of a gel.

EMILE E. HABIB.  
DAVID G. GREENLIE.

#### REFERENCES CITED

20 The following references are of record in the file of this patent:

#### UNITED STATES PATENTS

| Number    | Name           | Date          |
|-----------|----------------|---------------|
| 2,334,709 | Katzman et al. | Nov. 23, 1943 |
| 2,348,689 | Abrams et al.  | May 9, 1944   |